

# UNITED STATES PATENT OFFICE.

ROBERT C. TOTTEN, OF PITTSBURG, PENNSYLVANIA.

## COMPOSITION OF METAL.

No. 881,036.

Specification of Letters Patent.

Patented March 3, 1908.

Application filed June 8, 1907. Serial No. 377,866.

*To all whom it may concern:*

Be it known that I, ROBERT C. TOTTEN, a resident of Pittsburgh, in the county of Allegheny and State of Pennsylvania, have invented a new and useful Improvement in Composition of Metal; and I do hereby declare the following to be a full, clear, and exact description thereof.

My invention relates to a composition of chilling cast iron and to the manufacture of the same and the articles produced therefrom, its object being to provide from what are known as coal or coke irons, that is, pig metal smelted with coke or anthracite coal, what is known as a "chilling" cast iron, suitable for the manufacture of castings of great strength and fineness of grain, such as chilled castings, which have heretofore been made principally from what is known as charcoal iron. Charcoal pig iron has generally been considered a necessity for the making of such chilled castings, the generally understood reason for this being that it is the only pig metal that contains what is termed "combined carbon" in sufficient quantity to impart to the iron containing it the peculiarity of making a chilled surface when cast against a metal chill. One theory in regard to this combined carbon is that the carbon is chemically united or combined with the iron as distinguished from being present in graphitic form. While the demand for this charcoal pig iron has been constantly increasing, the production of the same has apparently reached its limit, largely on account of the cost of the charcoal necessary for smelting the same. By my invention I am able to produce from pig iron made by the coke and coal process, a chilling cast metal having practically the same properties as found in the charcoal pig iron, and thus to utilize a cheaper pig iron for the purpose and one of which there is abundant supply.

My invention consists, generally stated, in a new composition of "chilling" cast metal, consisting of coke or coal iron and carbid of silicon; the latter being the product of melting sand and carbon together in an electric furnace, its formula being  $SiC$ , and known to the trade as carborundum. It analyzes high in carbon, and when used with melted

cast coke or coal iron, gives to the metal the peculiar qualities ordinarily found in charcoal iron as above referred to.

In the manufacture of this chilling iron I 55 melt the coke or coal iron in any suitable way, preferably in an air furnace, and either before or after the metal is drawn from the furnace, I add to the melted iron the proper proportion of carbid of silicon to produce 60 the proper depth of chill which may be tested while the metal is still molten.

The ordinary coke or coal pig iron contains a large amount of graphitic carbon and a small proportion, sometimes only a trace, 65 of combined carbon. Carbid of silicon contains as high as 35% of carbon. I mix the coke or coal pig iron with carbid of silicon in suitable proportions in order to obtain the requisite amount of combined carbon in the 70 resultant casting iron, it being desired that this proportion shall be as much as one-quarter of one per cent. ( $\frac{1}{4}$  of 1%) of carbon for strong, fine grained castings, and as much as one-half of one per cent. ( $\frac{1}{2}$  of 1%) 75 or over for chilled rolls, car wheels, etc. For this purpose I can vary the amount of carbid of silicon in any desired proportion, being mixed together in any suitable way to produce a casting with suitable strength 80 and fineness of grain for a chilled roll car wheel and the like, the chill usually being from one-half inch to two inches in depth. As an illustration, using coal or coke iron with say one-quarter of one per cent. ( $\frac{1}{4}$  of 85 1%) combined carbon, and carbid of silicon containing 35% of carbon, a mixture would be produced by using 5% to 7% of such carbid of silicon that would contain  $1\frac{1}{2}$  to 2 per cent. of carbon producing a high chilling 90 iron. In this way I am able to produce a cast iron of fine grain and great strength, adapted to produce castings of the character referred to and especially chilled rolls, car wheels, etc., with a hard wearing surface 95 and the necessary strength back of the chilled surface in the body of the roll or car wheel. As the supply of charcoal iron is limited and the supply of ordinary coke or coal iron practically unlimited, I am thus 100 enabled to produce a cheap and suitable substitute for the ordinary charcoal iron.

What I claim is:

1. A new composition of chilling cast iron, consisting of coke or coal iron and carbid of silicon.
- 5 2. A new composition of chilling cast iron, consisting of coke or coal iron and carbid of silicon, containing combined iron and carbon, the composition containing at least one-

fourth of one per cent. ( $\frac{1}{4}$  of 1%) of combined carbon.

In testimony whereof, I the said ROBERT C. TOTTEN have hereunto set my hand.

ROBERT C. TOTTEN.

Witnesses:

JOHN R. KELLER,  
JOHN F. WILL.